# EUROPEAN PATENT SPECIFICATION

(11) **EP 0 515 673 B1**
(45) Date of publication and mention of the grant of the patent: **27.09.1995**
(21) Application number: 92903472.6
(22) Date of filing: 17.12.1991
(51) Int. Cl.: B63B 3/16

(54) **METAL PLATE ASSEMBLY FABRICATION SYSTEM**
VERFAHREN ZUR HERSTELLUNG VON METALLPLATTENSTRUKTUREN
SYSTEME DE FABRICATION D'UN ENSEMBLE COMPOSE DE PLAQUES METALLIQUES

(30) Priority: 21.12.1990 US 632346; 18.07.1991 US 732467
(43) Date of publication of application: 02.12.1992
(73) Proprietor: FALCON MARITIME VENTURES, L.P., Colorado Springs, CO 80906 (US)
(72) Inventor: JOHNSTON, Daniel, D., Port Townsend, Washington 98368 (US)
(74) Representative: Grünecker, Kinkeldey, Stockmair & Schwanhäusser Anwaltssozietät
(86) International application number: US9109324
(87) International publication number: WO9211178

(56) References cited:
- US-A- 2 251 621
- US-A- 4 744 320
- A GROUP OF AUTHORITIES 'Ship design and construction' 1969 , SOCIETY OF NAVALARCHITECTS AND MARINE ENGINEERS , NEW YORK

## Description

The invention relates to a method according to the preamble part of claim 1 and to a metal plate assembly according to claim 11.

US-A-4 744 320 discloses a method for fabricating a boat hull such as an aluminium plate boat hull. According to the disclosed method, a frame is provided to which hull plates along their longitudinal edges are bonded by tack and stitch weldings. Finally, the joints between adjacent hull plates are provided with continuous fillet weldings fully penetrating the joints. The hull plates bow outwardly. The space between the hull plates and the frame between the edges of the plates is filled with a foam. The amount of curvature that is induced into the plates by applying said method is limited.

It is a primary object of the invention to provide an improved fabrication method for a metal plate assembly as well as a metal plate assembly with increased torsional stiffness.

Said object can be achieved with the method as disclosed in claim 1.

Due to the transfer of sufficient heat during fillet welding, the outer skin of the plate is maintained in compression. The resulting metal plate assembly is stiff in torsion and can be analysed approximately as a compressively loaded cylinder. Having the metal plates on a supporting frame, e.g. to create a boat hull, it is possible to produce said boat hull lighter and less expensively than with the known method. The weight of the boat hull is then approximately 20% less and costs approximately 30% less to fabricate. This is in large part due to a great spacing between adjacent frame bulk heads. Furthermore, a wider range of hull shapes is possible in view of the increased plate bowing. This further reduces costs by reducing or eliminating conventional fairing steps. The higher stiffness in torsion allows the bulk heads to be placed further apart, and it is believed to maintain the fillet welds in compression, thereby reducing weld stress. Particularly, in the region of the bow, the method allows curves not previously feasible and which are deeper, more rounded and more suitable in an optimum hull shape.

Embodiments of the invention are described with the help of the drawings. In the drawings is
- Figure 1:: A side elevational view of a vessel hull,
- Figure 2:: A top, front and perspective view of the hull of Figure 1;
- Figure 3:: A perspective of a frame included in the hull of Figures 1 and 2,
- Figure 4:: A cross section in Figures 1 and 2,
- Figures 5, 6 and 7:: Enlarged views of portions of the cross section of Figure 4, and
- Figure 8:: A cross section of a second embodiment of a vessel hull.

Figures 1, 2 and 4 show various views of a vessel hull 10 which is configured as a boat hull, and in this example has an overall length of 24,3 m (80 feet) and a beam measured at the deck of 6,1 m (20 feet).

The outer surfaces of the hull 10 are formed by a pair of side plates 12, a pair of bottom plates 14, a pair of chine plates 15, and a top plate 16. A transom 18 extends between the opposed side plates 12 and bottom plates 14, and a superstructure 20 is positioned on the top plate 16, which forms the upper deck of the hull 10.

As described in U.S. -A-4,744,320 the plates 12, 14, 16 are preferably metal plates shaped to extend in uninterrupted fashion from the bow to the stern of the hull 10. Depending upon the size of the hull 10, the plates 12, 14, 16 may be either one piece, unitary plates, or they may alternately be fabricated from a plurality of component plates, as for example by welding. If the plates 12, 14, 16 are fabricated from component plates, the weld lines should preferably be ground and finished such that each of the plates 12, 14, 16 has many of the characteristics of a unitary plate.

As described below, the plates 12, 14, 15, 16 are assembled around a frame 40, which is shown in perspective view in Fig. 3. The frame 40 is a welded assembly which includes a longitudinally extending keel 42 and an array of parallel bulkheads 44. As best shown in Fig. 4, each of the bulkheads 44 in this embodiment includes a pair of bottom braces 46 which are welded at their inner ends to the keel 42, a pair of side braces 50 that are welded to the outer ends of the bottom braces 46, and a top brace 52 that extends between opposed side braces 54. As shown in Fig. 3, adjacent bulkheads 44 are braced one with respect to the next by longitudinal braces 54 that are preferably welded in place to the bottom, side and top braces. In this embodiment the braces 46, 50, 52, 54 are all formed as I-beams. In alternate embodiments it may be preferable to use other sections, such as T-shaped sections for some or all of the braces.

As pointed out below, the frame 40 is fabricated in stages, and the plates 12, 14, 16 are secured in place to the frame 40 as it is being fabricated. For this reason, Fig. 3 must be regarded as schematic, and the frame 40 is not completely assembled as shown in Pig. 3 before the plates 12, 14, 16 are secured in place.

The hull 10 is preferably fabricated as follows. First, the two bottom braces 46 of each bulkhead 44 are securely welded in the desired geometry to the keel 42. Similarly, the side braces 50 are securely welded in place to the respective bottom braces 46. At this stage in the fabrication of the hull 10 the frame 40 is preferably inverted, with the keel 42 uppermost, and the ends of the side braces 50 that will be secured to the top brace 52 are positioned at or adjacent ground level. A suitable fixture (not shown) is used to hold the partially assembled frame 40 in position.

The next step in the assembly of the hull 10 is to stitch weld the bottom plates 14, the chine plates 15, and the side plates 12 in place. The locations of the stitch welds are identified by the reference numerals 60 in Fig. 4, and they are positioned on the inside of the hull 10, between the bottom plates 14 and the keel 42, between adjacent edges of the bottom plates 14 and the chine plates 15, and between adjacent edges of the chine plates 15 and the side plates 12. Additionally, the stitch welding secures the plates 12, 14, 15 at their longitudinal edges securely to the bottom braces 46 and the side braces 50.

The purpose of the stitch welds 60 is to immobilize the longitudinal edges of the side and bottom plates 12, 14 and to prevent the longitudinal edges from moving away from one another. In this preferred embodiment, the stitch welds are approximately 6,35 mm (1/4 inch) in width, and approximately 101,6 mm (4 inches) in length. Adjacent stitch welds are separated by an unwelded length of approximately 203,2 mm (8 inches). Because the stitch welds 60 are confined to the longitudinal edges of the side and bottom plates 12, 14, the central portions of the side and bottom plates 12, 14 are free to move away from the braces 46, 50.

Once the side, bottom and chine plates 12, 14, and 15 have been stitch welded in place, fillet welds 62 are used to secure the plates 12, 14 and 15 permanently together to form the lower portion of the hull 10. The fillet welds 62 should preferably have a penetration of greater than 50%, and a full penetration fillet weld will often be preferred.

Fig. 5 shows an enlarged view of the portion of the bottom plates 14 adjacent to the keel 42. The included angle A between the longitudinal edges of the plates 14 is preferably between 45 and 90°. Fig. 6 shows an enlarged view of the welds at the chine plate 15. The angle between the bottom plate 14 and the chine plate 15 will be referred to as the inner chine angle B and is preferably about 30°. The outer longitudinal edge of the chine plate 15 is preferably bevelled as shown in Fig. 6 to define an outer chine angle C of approximately 30° between the chine plate 15 and the side plate 12.

The fillet welds 62 are preferably formed in an uninterrupted fashion from one end of the hull 10 to the other. It has been discovered that, when welding conditions are chosen properly, the heat of welding will cause the plates 12, 14 to bow outwardly so as to define a convex outer surface and a concave inner surface. The plates 12, 14 are not secured to the bulkheads 44 intermediate their longitudinal edges, and they are therefore free to bow outwardly as the plates 12, 14 are heated in the welding operation. In general, it has been discovered that the more heat that is applied during welding the fillet welds 62, the greater the curvature that is induced into the plates 12, 14.

Residual stress measurements on test samples indicate that when the plates 12, 14 cool after formation of the fillet welds 62, they retain an outwardly bowed configuration, with at least the central portion the outer skin 24 of the plates 12, 14 in compression along an axis extending along the span between the fillet welds 62 (i.e., in the plane of Figure 4). Without intending to be bound by any theory of operation, it is believed that because the longitudinal edges of the plates 12, 14 are stitch welded in place, the thermal elongation of the plates 12, 14 during formation of the fillet welds 62 applies sufficient tensile forces to the outer skin 24 so as to increase the effective width of the plates 12, 14 at the outer skin 24. Then, when the plates 12, 14 cool to ambient temperature, this increased width of the plates 12, 14 causes the outer skin 24 to be in compression, even when the same ambient pressure is applied to both the convex outer surface and the concave inner surface of the plates 12, 14.

As pointed out above, the degree of bowing of the plates 12, 14 has surprisingly been found to depend upon the amount of heat applied to the plates 12, 14 during formation of the fillet welds 62. In this preferred embodiment fillet welds are applied in a total of three passes at the keel angle A, while only Two passes are used at the inner and outer chine angles B, C.

Once the side and bottom plates 12, 14 have been fillet welded in place, the partially assembled hull is then inverted to place the keel 42 in the lower most position. The top braces 52 are then welded in place between opposed ones of the side braces 50, and the top plate 16 is then installed by first stitch welding it in place along its inner longitudinal edges, as described above. Then the top plate 16 is fillet welded in place using preferably only a single pass at the deck angle D. Thermal deformation associated with formation of this fillet weld causes the top plate 16 to bow away from the top brace 52.

At this point, fabrication and assembly of the plates 12, 14, 15, 16 and the bulkheads 44 has been completed. The transom 18 and superstructure 20 are now added in the conventional manner, and the frame 40 is completed by welding the longitudinal braces 54 between adjacent bulkheads 44. The longitudinal braces 54 are preferably positioned approximately 19,05 mm (3/4 inch) from the inner surface of the plates 12, 14, 16 and securely welded in place to the bulkheads 44 only.

The hull 10 is now allowed to stand for 24 hours to allow temperature differences to equilibrate. The next step is to apply a foam between the frame 40 and the plates 12, 14, 16. In particular, the foam spreads loads such as the shock associated with water impact efficiently from the plates 12, 14, 16 to the frame 40.

The following information is provided to define the presently preferred embodiment of this invention, and is only intended by way of illustration. In this embodiment the plates 12, 14, 15, 16, transom 18, and frame 40 are all formed of 5000 series aluminum or stronger, such as 5086H11G or 5086H32. The preferred dimensions for the elements 12 through 20 are defined in Table 1.

**Table 1**

| | Thickness mm (Inches) | Width m |
|---|---|---|
| Side plate 12 | 6,35 (1/4) | 2,44 (8') |
| Bottom plate 14 | 9,525 (3/8) | 3,048 (10') |
| Chine plate 15 | 9,525 (3/8) | |
| Top plate 16 | 4,762 (3/16) | 6,096 (20') |
| Transom 18 | 9,525 (3/8) | 6,096 (20') |
| Keel 42 | 19,05 (3/4) | 0,203 8" |

The bulkheads 44 are preferably spaced about 1,524 m (5 feet) apart and have a preferred web depth of 203 mm (8 inches) and flange width of 101,6 mm (4 inches). 6,35 mm or 7,94 mm (One quarter or 5/16 inch) thick plate can be used. The longitudinal braces 54 are preferably spaced 0,76 m (2-1/2 feet) apart and are fabricated from 6,35 mm (1/4 inch) thick plate aluminum with a web depth of 152,4 mm (6 inches) and a flange width of 101,6 mm (4 inches). Of course prefabricated I beams may be used if desired. The presently preferred sealant foam is General Electric Silglaze N SCS2501 silicone sealant. The presently preferred welding parameters for formation of the fillet welds 62 include use of a MIG welding gun operating at 140 A (amps) using 5356 filler rod having a diameter of 1,19 mm (3/64 inch). The fillet weld is preferably formed slowly at a rate no less than 82s/m (25 seconds per foot). As explained above, multiple passes are used until the desired degree of plate curvature is reached. In this example, the maximum bowing (measured at the center of the plate) is approximately 63,5 mm (2-1/2) inches away from the bulkhead 44 at the side and bottom plates 12, 14, and approximately 38,1 mm (1-1/2 inches) away from the bulkhead 44 at the top plate 16.

The preferred embodiment described above uses the heat of welding the fillet welds 62 to induce an unusually large amount of curvature into the plates 12, 14. Figure 4 defines the dimensions H and S that will be used as a measure of the thermally induced curvature. As shown in Figure 4, S is the span between the fillet welds 62, and is a measure of the unsupported width of the plate 12, 14 between the stitch welds 60. H is the maximum height by which the plate 12, 14 moves outwardly as a result of the formation of the fillet welds 62, as measured at the center of the plate 12, 14 after the plate 12, 14 has returned to equilibrium temperature. The ratio H/S indicates the thermally induced height of curvature per unit span, and this ratio provides a measure of the thermally induced curvature of the plates. Table 1 shows the valves for H, S, and H/S for the plates 12 and 14:

**TABLE 1**

| Plate | H mm (inch) | S mm (inch) | H/S |
|---|---|---|---|
| 12 | 63,5 (2.5) | 2438,4 (96) | 0.026 |
| 14 | 63,5 (2.5) | 3048 (120) | 0.021 |

By way of comparison, the maximum thermally induced curvature achieved with the process of U.S.-A-4,744,320 was much less than that of the plates 12, 14; with the process of the '320 patent was achieved H=6,35 mm, S=1,22 m, H/S=0.0052. There is no suggestion in the '320 patent that it is possible to achieve thermally induced curvatures greater than H/S=0.01, preferably greater than H/S=0.015, and most preferably greater than H/S=0.02.

The method of this invention produces a hull which is lighter and less expensive than that produced by the method of U.S.-A-4,744,320. The weight of the hull 10 is approximately 20% less than that obtainable with the method of the '320 patent and costs approximately 30% less to fabricate. This is in large part due to the greater spacing between adjacent bulkheads made possible with this invention. Furthermore, a wider range of hull shapes is possible in view of the increased plate bowing made possible by the present invention. This further reduces costs by reducing or eliminating conventional fairing steps.

Because the outer skin 24 of the plates 12, 14, 16 is maintained in compression, the resulting hull is stiff in torsion and can be analyzed approximately as a compressively loaded cylinder. This allows the bulkheads to be placed farther apart, and it is believed to maintain the fillet welds in compression, thereby reducing weld stress. Particularly in the region of the bow, the present invention allows curves not previously feasible, and which are deeper, more rounded and more suitable to an optimum hull shape.

Fig. 8 shows a cross-sectional view of a hull 110 which incorporates a second preferred embodiment of this invention. The hull 110 is for a rigid inflatable boat and includes a pair of bottom plates 112 and a top plate 114. The bottom plates 112 are secured together at a keel 120, and the hull 110 supports pontoon supports 116 which in turn support pontoons 118. The hull 110 is a shallow draft boat having an overall length of 9,144 m (30 feet), a maximum beam of 2,54 m (100 inches), and a hull depth of about 0,508 m (20 inches). In applications such as the hull 110, a frame of the type described above may be optional. That is, temporary fixtures may be used to secure the plates in place during fillet welding, eliminating the need for a permanent internal frame.

The present invention is not limited to use in fabricating boat hulls, but can also be used to fabricate other types of hulls such as airplane or submarine hulls. The invention is not limited to use with aluminum plates, but can also be used with other types of metals, and it is not limited to relatively thick plate of the type described above. Thinner plates down to about 14 gauge or 3,175 mm (0.125") in thickness can be used for applications such as aircraft hulls, and thicker plates can be used for applications such as submarine hulls.

Furthermore, the present invention is not limited to use in fabricating vessel hulls, but can also be used to fabricate other types of metal plate assemblies, such as boat superstructures that require complexly curved surfaces.

## Claims

1. A method of forming at least a portion of a metal plate assembly comprising the following steps :
(a) providing a plurality of metal plates (12,14,16;15) at least a first one (12,14,16) of said plates having a pair of spaced longitudinal edges;
(b) securing the longitudinal edges of the first plate (12,14,16) in position to prevent outward movement thereof;
(c) welding the longitudinal edges of the first plate (12,14,16;15) in position to cause the welded first plate (12,14,16) to bow outwardly between the longitudinal edges such that said welded first plate defines convex outer and concave inner surfaces,
**characterised in that**
the longitudinal edges of the first plate (12,14,16) are welded in position with sufficient heating of the welded first plate to cause the welded first plate (12,14,16) to bow outwardly between the longitudinal edges such that the first plate defines a ratio H/S greater than 0,01, where S is the span between opposed longitudinal edges of the first plate (12,14,16) and H is the maximum amount by which the first plate moves outwardly at a result of the welding step.

2. A method as in claim 1, **characterised in that** at least a central portion of the convex outer surface of the first plate (12,14,16) is placed in compression along an axis extending along the span when the welded first plate cools to ambient temperature and ambient pressure on the inner surface is equal to ambient pressure on the outer surface.

3. Method as in claim 1, **characterised in that** the longitudinal edges of the first plate (12,14,16) are welded in position with a step of forming fillet welds (62) having a penetration of at least 50% along substantially the entire length of the welded longitudinal edges, the fillet welds (62) being formed preferably in one pass or in more than one pass.

4. Method as in claim 3, **characterised by** the following steps:
(b1) providing an internal frame (40); and
(b2) welding the first plate (12,14,16) to the frame (40) by stitch welds (60) from the side of the frame (40) and adjacent the longitudinal edges to secure the longitudinal edges of the first plate (12,14,16) in position on the frame (40).

5. Method as in claim 4, **characterised in that** welding the first plate (12,14,16) to the frame (40) by stitch welds (60) to secure the longitudinal edges of the first plate in position comprises the step of avoiding any interconnection between the first plate (12,14,16) and the frame (40) intermediate longitudinal edges prior to welding the longitudinal edges of the first plate in position with sufficient heating of the welded first plate to cause the welded first plate to bow outwardly such that the ratio H/S becomes greater than 0,01. plate to cause the welded first plate to bow outwardly such that the ratio H/S becomes greater than 0,01.

6. Method as in at least one of claims 1 to 5, **characterised in that** a foam is introduced between the frame (40) and the concave inner surface of the bowed first plate (12,14,16).

7. Method as in claim 1, **characterised in that** the first bowed plate defines a ratio H/S greater than 0,015.

8. Method as in claim 1, **characterised in that** the bowed first plate (12,14,16) defines a ratio H/S greater than 0,02.

9. Method as in claim 1, **characterised in that** the plates (12,14,16;15) are formed of an aluminium alloy.

10. Method as in at least one of claims 1 to 9, **characterised in that** the plates (12,14,16;15) are hull plates, and that the hull plates' longitudinal edges are secured in position in a configuration suitable for a boat hull (10).

11. Metal plate assembly produced by the method of claim 10.

## Patentansprüche

1. Verfahren zum Formen wenigstens eines Abschnittes einer Metallplatteneinrichtung, das folgende Schritt umfaßt:
a) Bereitstellen einer Vielzahl von Metallplatten (12, 14, 16; 15), von denen wenigstens eine erste (12, 14, 16) ein Paar beabstandeter Längsränder aufweist;
b) Festlegen der Längsränder der ersten Platte (12, 14, 16) in ihren Positionen, um deren Bewegung nach außen zu verhindern;
c) Festschweißen der Längsränder der ersten Platte (12, 14, 16; 15) in Position, um die geschweißte erste Platte (12, 14, 16) zu veranlassen, sich zwischen den Längsrändern nach außen zu biegen, derart, daß die geschweißte erste Platte konvexe äußere und konkave innere Flächen definiert,
**dadurch gekennzeichnet**, daß die Längsränder der ersten Platte (12, 14, 16) in ihren Positionen unter ausreichender Erwärmung der verschweißten ersten Platte geschweißt werden, um die geschweißte erste Platte (12, 14, 16) zu veranlassen, sich zwischen den Längsrändern derart nach außen zu biegen, daß die erste Platte ein Verhältnis (H/S) größer als 0,01 definiert, wobei (S) die Spannweite zwischen gegenüberliegenden Längsrändern der ersten Platte (12, 14, 16) und (H) das maximale Ausmaß ist, um das sich die erste Platte als Resultat der Schweißung nach außen bewegt.

2. Verfahren nach Anspruch 1, **dadurch gekennzeichnet**, daß zumindest ein zentraler Bereich der konvexen äußeren Fläche der ersten Platte (12, 14, 16) unter Kompression entlang einer Achse plaziert ist, die sich entlang der Spannweite erstreckt, sobald die geschweißte erste Platte auf Umgebungstemperatur abkühlt und der Umgebungsdruck auf der inneren Fläche gleich dem Umgebungsdruck auf der äußeren Fläche ist.

3. Verfahren nach Anspruch 1, **dadurch gekennzeichnet**, daß die Längsränder der ersten Platte (12, 14, 16) in ihren Positionen unter Formung von Kehlnahtschweißungen (62) verschweißt sind, die eine Eindringtiefe von zumindest 50% entlang im wesentlichen der gesamten Länge der geschweißten Längsränder haben, wobei die Kehlnahtschweißungen (62) vorteilhafterweise in einem Zug oder in mehr als einem Zug geformt werden.

4. Verfahren nach Anspruch 3, **gekennzeichnet durch** die folgenden Schritte:
b1) Bereitstellen eines inneren Rahmens (40); und
b2) Anschweißen der ersten Platte (12, 14, 16) am Rahmen (40) durch Heftschweißungen (60) von der Seite des Rahmens her und benachbart zu den Längsrändern, um die Längsränder der ersten Platte (12, 14, 16) in ihren Positionen an dem Rahmen (40) festzulegen.

5. Verfahren nach Anspruch 4, **dadurch gekennzeichnet**, daß das Anschweißen der ersten Platte (12, 14, 16) am Rahmen (40) mit den Heftschweißungen (60) zum Festlegen der Längsränder der ersten Platte in ihren Positionen den Schritt umfaßt, jegliche Zwischenverbindungen zwischen der ersten Platte (12, 14, 16) und dem Rahmen (40) zwischen Längsrändern zu vermeiden, ehe die Längsränder der ersten Platte mit ausreichender Erwärmung der geschweißten ersten Platte geschweißt werden, um die geschweißte erste Platte zu veranlassen, sich so weit nach außen zu biegen, daß das Verhältnis (H/S) größer als 0,01 wird.

6. Verfahren nach wenigstens einem der Ansprüche 1 bis 5, **dadurch gekennzeichnet**, daß zwischen den Rahmen (40) und die konkave innere Fläche der gebogenen ersten Platte (12, 14, 16) ein Schaum eingeführt wird.

7. Verfahren nach Anspruch 1, **dadurch gekennzeichnet**, daß die gebogene Platte ein Verhältnis (H/S) größer als 0,015 definiert.

8. Verfahren nach Anspruch 1, **dadurch gekennzeichnet**, daß die gebogene erste Platte (12, 14, 16) ein Verhältnis (H/S) größer als 0,02 definiert.

9. Verfahren nach Anspruch 1, **dadurch gekennzeichnet**, daß die Platten (12, 14, 16; 15) aus einer Aluminiumlegierung geformt sind.

10. Verfahren nach wenigstens einem der Ansprüche 1 bis 9, **dadurch gekennzeichnet**, daß die Platten (12, 14, 16; 15) Hüllplatten sind, und daß die Längsränder der Hüllplatten in einer für eine Bootshülle (10) passenden Konfiguration in ihren Positionen festgelegt sind.

11. Metallplatteneinrichtung, die mit dem Verfahren gemäß Anspruch 10 hergestellt ist.

## Revendications

1. Procédé de formage d'au moins une partie d'un ensemble composé de plaques métalliques, comprenant les étapes consistant à :
(a) fourniture d'une pluralité de plaques métalliques (12, 14, 16 ; 15), au moins une première (12, 14, 16) desdites plaques ayant une paire de bords longitudinaux espacés ;
(b) fixer en place les bords longitudinaux de la première plaque (12, 14, 16) afin d'empêcher un déplacement vers l'extérieur de ceux-ci ;
(c) souder les bords longitudinaux de la première plaque (12, 14, 16 ; 15) en place pour amener la première plaque soudée (12, 14, 16) à se courber vers l'extérieur entre les bords longitudinaux de sorte que ladite première plaque soudée définisse des surfaces extérieure convexe et intérieure concave,
caractérisé en ce que
les bords longitudinaux de la première plaque (12, 14, 16) sont soudés en place avec un chauffage suffisant de la première plaque soudée pour amener la première plaque soudée (12, 14, 16) à se courber vers l'extérieur entre les bords longitudinaux de sorte que la première plaque définisse un rapport H/S supérieur à 0,01, où S représente la portée entre les bords longitudinaux opposés de la première plaque (12, 14, 16) et H représente la valeur maximale avec laquelle la première plaque se déplace vers l'extérieur à la suite de l'étape de soudage.

2. Procédé selon la revendication 1, caractérisé en ce qu'au moins une partie centrale de la surface extérieure convexe de la première plaque (12, 14, 16) est placée en compression le long d'un axe qui s'étend suivant la portée lorsque la première plaque soudée refroidit à la température ambiante et lorsque la pression ambiante sur la surface intérieure est égale à la pression ambiante sur la surface extérieure.

3. Procédé selon la revendication 1, caractérisé en ce qu'au moins les bords longitudinaux de la première plaque (12, 14, 16) sont soudés en place avec une étape de formation de soudures en angle (62) ayant une pénétration d'au moins 50% sensiblement sur toute la longueur des bords longitudinaux soudés, les soudures en angle (62) étant formées de préférence en une seule passe ou en plus d'une seule passe.

4. Procédé selon la revendication 3, caractérisé par les étapes consistant à :
(b1) fournir une ossature intérieure (40) ; et
(b2) souder la première plaque (12, 14, 16) à l'ossature (40) par des soudures par points (60) depuis le côté de l'ossature (40) et de façon adjacente aux bords longitudinaux pour fixer les bords longitudinaux de la première plaque (12, 14, 16) sur l'ossature (40).

5. Procédé selon la revendication 4, caractérisé en ce que le soudage de la première plaque (12, 14, 16) à l'ossature (40) par des soudures par points (60) de manière à fixer en place les bords longitudinaux de la première plaque comprend l'étape consistant à éviter toute communication entre la première plaque (12, 14, 16) et ladite ossature (40) entre les bords longitudinaux avant le soudage des bords longitudinaux de la première plaque avec un chauffage suffisant de la première plaque soudée pour amener celle-ci à se courber vers l'extérieur de sorte que le rapport H/S devienne supérieur à 0,01.

6. Procédé selon au moins l'une des revendications 1 à 5, caractérisé en qu'une mousse est introduite entre l'ossature (40) et la surface intérieure concave de la première plaque courbée (12, 14, 16).

7. Procédé selon la revendication 1, caractérisé en ce que la première plaque courbée définit un rapport H/S supérieur à 0,015.

8. Procédé selon la revendication 1, caractérisé en ce que la première plaque courbée (12, 14, 16) définit un rapport H/S supérieur à 0,02.

9. Procédé selon la revendication 1, caractérisé en ce que les plaques (12, 14, 16 ; 15) sont formées d'un alliage d'aluminium.

10. Procédé selon au moins l'une des revendications 1 à 9, caractérisé en ce que les plaques (12, 14, 16 ; 15) sont des plaques de bordé, et en ce que les bords longitudinaux des plaques de bordé sont fixés en place dans une configuration adaptée à une coque (10) de bateau.

11. Ensemble composé de plaques métalliques réalisé par le procédé de la revendication 10.
